

# United States Patent Office

3,188,204  
Patented June 8, 1965

1

3,188,204

## NICKEL-ALLOY

Claude R. Bishop, Niagara Falls, and William J. Boesch, Utica, N.Y., assignors to Union Carbide Corporation, a corporation of New York  
No Drawing. Filed Apr. 8, 1963, Ser. No. 271,488  
15 Claims. (Cl. 75—170)

This invention relates to a nickel-base alloy characterized by stability in oxidizing environments and by superior creep rupture properties at elevated temperatures.

Progress in the field of hypersonic aircraft and missiles has brought to light a number of problems relating to materials of construction. One such problem, to which no satisfactory solution has been evidenced in the past, is that of aerodynamic heating, i.e., heating caused by the friction of the atmosphere on the surface of an object travelling at high speeds. This phenomenon is associated with aircraft which operate at or near supersonic speeds. This particular problem is even more pronounced when the object is a missile or other space vehicle the trajectory of which carries it out of the atmosphere and back again. Re-entry into the atmosphere at hypersonic speeds subjects the outer surface of the object to extremely rapid heating and substantial stress. It is obvious that there is a present need for alloys which are capable of withstanding these extreme conditions.

Another problem encountered in connection with missiles is the need for a material which is suitable for use in oxidizing environments, e.g., fuming nitric acid which is used to oxidize fuels in rocket engines.

The problem of oxidation resistance is not unique to the missile field. Another field where stability in corrosive environments is important is in the construction of chemical processing equipment. In this particular field corrosion resistance combined with strength and ductility is of primary importance.

Moreover to be useful for such applications as the outer skin of a missile, or a component of a gas turbine these alloys must be amenable to known methods of fabrication and forming.

It is therefore an object of this invention to provide a nickel-base alloy which exhibits superior creep-rupture properties at elevated temperatures.

It is another object of the invention to provide a nickel-base alloy which possesses a high degree of stability to corrosion when exposed to oxidizing environments at elevated temperatures.

It is a further object of the invention to provide a nickel-base alloy which combines superior creep-rupture resistance and which can be forged and rolled into various forms and thin sheets.

These and other related objects are achieved by providing an alloy comprising, along with incidental impurities, at least 25 weight percent nickel, 1 to 25 weight percent tantalum, 20 to 50 weight percent tungsten, and a maximum of 0.5 weight percent carbon.

Additional highly desirable alloys are obtained by the addition, to the above composition, of selected amounts of at least one metal chosen from the group comprising, iron, aluminum, molybdenum, and chromium.

Iron, aluminum, molybdenum, and chromium in selected amounts have been found to exert a desirable effect on one or more of the characteristics of the herein described alloy. By varying and adjusting the amounts of the various additive metals highly desirable combinations of properties, such as workability, high temperature strength, corrosion resistance, and the like can be achieved.

In general the additive metals are employed in amounts within the following ranges: iron, from about 4 to about

2

12 weight percent; aluminum, from about 1 to about 5 weight percent; molybdenum, from about 5 to about 15 weight percent; and chromium, from about 8 to about 20 weight percent. The above stated ranges may conveniently be referred to as "selected amounts" of the particular metal.

An alloy which is particularly corrosion resistant comprises 24 to 50 weight percent tungsten, 5 to 15 weight percent tantalum, at least 40 weight percent nickel, a maximum of 0.15 weight percent carbon, incidental impurities, and at least one additive selected from the group comprising 4 to 10 weight percent iron, 1 to 5 weight percent aluminum, 5 to 15 weight percent molybdenum, and 8 to 15 weight percent chromium.

An alloy evidencing enhanced creep-rupture resistance comprises, along with normally present impurities, 20 to 45 weight percent tungsten, 1 to 20 weight percent tantalum, at least 35 weight percent nickel, a maximum of 0.15 weight percent carbon and at least one additive selected from the group comprising 1 to 2 weight percent aluminum, 8 to 20 weight percent chromium, and 5 to 15 weight percent molybdenum.

The most preferred alloy satisfying the above-mentioned corrosion-resistance objects comprises 24 to 50 weight percent tungsten, 5 to 15 weight percent tantalum, up to 10 weight percent iron, up to 5 weight percent aluminum, up to 15 weight percent molybdenum, up to 15 weight percent chromium, a maximum of about 0.5 weight percent carbon, the balance at least 40 weight percent nickel and the remainder incidental impurities.

The most preferred alloy satisfying the above-mentioned creep-rupture resistance at high heating rate and at high temperatures comprises 20 to about 45 weight percent tungsten, 1 to 20 weight percent tantalum, up to about 2 weight percent aluminum, up to about 20 weight percent chromium, up to about 15 weight percent molybdenum, a maximum of about 0.5 weight percent carbon, the balance at least 35 weight percent nickel and the remainder incidental impurities.

Creep is the flow or plastic deformation of metals held at stresses lower than the normal yield strength. The conventional creep-rupture test normally consists of submitting a specimen to a constant tensile load or stress at a constant ambient temperature and up to about 1000° C. for given periods of time and measuring the total creep in inches per inch at given times. These parameters are plotted against one another to obtain a tensile creep curve. Tests of this type are especially useful in ascertaining the creep-rupture characteristic of metals at ambient temperature and up to about 1000° C. because the time of application of stress is very long before rupture is experienced. The final result of the above creep-rupture test will be a creep-rupture index denoting minute fractions of an inch creep per inch of original specimen length per thousands of hours at ambient temperatures.

An artisan selects a proper material by correlating a fixed permissible deformation and required service time with the creep-rupture index of tested materials to decide which materials are amenable to his specific purpose.

The conventional creep-rupture test has been used herein at an elevated temperature of approximately 1000° C. A creep-rupture index was obtained, which due to the short total life of the specimen before rupture, is of necessity expressed in total hour-life before rupture.

Conventional tests, however, are obviously unsuited to properly evaluate materials which are to be subjected to the severe conditions imposed by re-entry of a missile into the atmosphere for example. Materials operating under these conditions are shocked by an abrupt application of

high temperature, pressure and rapid heating. Their behavior under these conditions cannot be predicted by the results of conventional creep-rupture tests; therefore, special tests have been devised which are characterized by short duration, high temperature, and rapid heating rates which closely simulate the type of conditions actually encountered by missiles and the like. Since extremely high temperatures are employed in the special tests, the creep-rupture life in these tests is considerably reduced for all metals and is expressed in total life-minutes before rupture. The alloys of the present invention exhibit surprising creep-rupture resistance under the special creep-rupture tests.

The superior corrosion resistant properties of the alloy of this invention to the corrosive attack of highly oxidizing media is evidenced by tests in which samples of the alloy were subjected to the action of several corrosive solutions such as boiling, fuming nitric acid, and its condensate. The results of these tests are set forth in Table I. These samples were subjected to boiling fuming nitric acid condensate for an average of at least three 48-hour periods. The remainder of the data indicates that the alloy of this invention also has improved corrosion re-

sistance to reducing media such as hydrochloric acid and moderately low concentrations of sulfuric acid.

Included within Table I are test results obtained by subjecting commercially available alloys to the same environments as the alloy of this invention.

From the data presented in Table I, it may be seen that the alloy composition range for maximum corrosion resistance is between about 25 to 50 weight percent tungsten, 5 to 15 weight percent tantalum and the balance nickel and incidental impurities, with the alloy containing a minimum of about 40 weight percent nickel.

The stress-rupture properties of the alloy of this invention were determined under conditions of rapid heating. The specimens were heated to a testing temperature of about 2300° F. at a rate approximately 150° F. per second during which time they were subjected to various amounts of stress. The results of these tests are set forth in Table II, III, IV and V. The alloys of this invention, under conditions of rapid heating, possessed stress-rupture properties far superior to prior art alloys. The results of rapid-heating rate, creep-rupture tests on prior art alloys are included in Table VI. The alloys of Table II, III, IV, V and VI contain incidental impurities.

Table I

| Composition, weight percent                 |          |       |       | Boiling fuming nitric acid condensate | Mils per year           |                       |      |       |                 |                          |  |
|---------------------------------------------|----------|-------|-------|---------------------------------------|-------------------------|-----------------------|------|-------|-----------------|--------------------------|--|
| W                                           | Ni       | Ta    | C     |                                       | Boiling 65% nitric acid | Boiling sulfuric acid |      |       | Boiling 20% HCl | Boiling 10% chromic acid |  |
|                                             |          |       |       |                                       |                         | 10%                   | 30%  | 55%   |                 |                          |  |
| 4.6                                         | Rem----- | 9.84  | 0.002 | 2,100                                 | 9,970                   | 183                   | 361  | 4,300 | 6,600           | 80.1                     |  |
| 10.44                                       | Rem----- | 11.05 | 0.003 | 420                                   | 9,780                   | 109                   | 523  | 569   | 1,730           | 64.6                     |  |
| 14.61                                       | Rem----- | 9.95  | 0.004 | 50.3                                  | 7,600                   | 498                   | 792  | 388   | 1,550           | 71.5                     |  |
| 25.05                                       | Rem----- | 9.80  | 0.001 | 5.0                                   | 2,510                   | 117                   | 56.5 | 240   | 1,130           | 94.7                     |  |
| 23.76                                       | Rem----- | 4.77  | 0.003 | 1.51                                  | 622.0                   | 15.8                  | 57.3 | 68.0  | 549             | 437                      |  |
| 24.00                                       | Rem----- | 10.64 | 0.040 | 0.57                                  | 3.43                    | 8.9                   | 23.8 | 63.1  | 525             | 53.6                     |  |
| 24.96                                       | Rem----- | 15.61 | 0.010 | 0.25                                  | 1.45                    | 6.13                  | 15.8 | 40.0  | 452             | 33.7                     |  |
| 31.52                                       | Rem----- | 21.01 | 0.026 | -----                                 | 23.1                    | 21.6                  | 52.2 | 26.8  | 251             | 174                      |  |
| 33.68                                       | Rem----- | 4.50  | 0.026 | 1.30                                  | 16.7                    | 19.8                  | 60.5 | 16.0  | 407             | 79.8                     |  |
| 46.01                                       | Rem----- | 9.03  | 0.068 | 0.59                                  | 3.66                    | 12.2                  | 18.4 | 44.0  | 436             | 76.5                     |  |
| 42.54                                       | Rem----- | 5.70  | 0.025 | 0.57                                  | 4.19                    | 5.57                  | 29.7 | 16.9  | 355             | 117                      |  |
|                                             |          | 11.12 | 0.014 | 0.24                                  | 1.73                    | 19.5                  | 20.4 | 51.0  | 385             | 81.1                     |  |
| Commercially available alloy                |          |       |       |                                       |                         |                       |      |       |                 |                          |  |
| 0.07, 18 Cr., 8 Ni., balance iron           |          |       |       | 1,260                                 | 10.0                    | 43.0                  | 38.0 | 143   |                 |                          |  |
| 20 Cr. 29 Ni., 2.0 Mo., 3 Cu., balance iron |          |       |       |                                       |                         |                       |      |       |                 |                          |  |

Table II

| Percent W | Percent Ta | Percent Ni | Percent C | Stress, p.s.i. at 1,250° C. |             |       |             |       |             |       |             |
|-----------|------------|------------|-----------|-----------------------------|-------------|-------|-------------|-------|-------------|-------|-------------|
|           |            |            |           | 3,000                       |             | 4,000 |             | 5,000 |             | 6,000 |             |
|           |            |            |           | Min.                        | Percent El. | Min.  | Percent El. | Min.  | Percent El. | Min.  | Percent El. |
|           |            |            |           |                             |             |       |             |       |             |       |             |
| 25.89     | 4.77       | Bal-----   | 0.040     | 71.3                        | 7.0         | 19.9  | 6.8         | ----- | -----       | 2.5   | 7.5         |
| 25.05     | -----      | Bal-----   | 0.008     | -----                       | -----       | 26.4  | 6.5         | 15.5  | 6.5         | 5.3   | 6.5         |
| 29.40     | -----      | Bal-----   | 0.006     | 57.8                        | 7.5         | 17.3  | 7.0         | ----- | -----       | 2.0   | 9.0         |
| 30.04     | -----      | Bal-----   | 0.027     | 42.1                        | 6.0         | 12.4  | 6.0         | ----- | -----       | ----- | -----       |
| 31.52     | 4.50       | Bal-----   | 0.026     | 57.5                        | 5.3         | 20.1  | 6.0         | 5.4   | 4.5         | 10.5  | 19.5        |
| 46.01     | 5.70       | Bal-----   | 0.025     | -----                       | -----       | 57.6  | 11.0        | 47.7  | -----       | ----- | 9.5         |

Table III

| Percent W | Percent Ta | Percent Ni | Percent C | Stress, p.s.i. at 1,250° C. |             |       |             |       |             |       |             |
|-----------|------------|------------|-----------|-----------------------------|-------------|-------|-------------|-------|-------------|-------|-------------|
|           |            |            |           | 2,000                       |             | 3,000 |             | 4,000 |             | 5,000 |             |
|           |            |            |           | Min.                        | Percent El. | Min.  | Percent El. | Min.  | Percent El. | Min.  | Percent El. |
|           |            |            |           |                             |             |       |             |       |             |       |             |
| 4.67      | 9.84       | Bal-----   | 0.002     | 106.3                       | 10.0        | 11.1  | 10.0        | 5.6   | 11.0        | ----- | -----       |
| 10.44     | 11.05      | Bal-----   | 0.003     | 126.6                       | 7.5         | 23.7  | 9.5         | 5.8   | 8.5         | ----- | -----       |
| 14.61     | 9.95       | Bal-----   | 0.004     | -----                       | -----       | 47.3  | 9.3         | 15.8  | 9.5         | 4.10  | 8.5         |
| 20.44     | 9.80       | Bal-----   | 0.001     | -----                       | -----       | 73.4  | 7.3         | 25.2  | 9.5         | ----- | -----       |
| 22.46     | 9.22       | Bal-----   | 0.024     | -----                       | -----       | ----- | -----       | 24.3  | 7.5         | 10.1  | 6.5         |
| 23.76     | 7.94       | Bal-----   | 0.004     | -----                       | -----       | ----- | -----       | 36.3  | 7.8         | 14.0  | 7.5         |
|           | 10.64      | Bal-----   | 0.040     | -----                       | -----       | 153.9 | 6.0         | 45.9  | 6.3         | ----- | 5.1         |

Table IV

| Percent<br>Ta | Percent<br>W | Percent<br>Ni | Percent<br>C | Stress, p.s.i. at 1,250° C. |                |       |                |       |                |       |                |
|---------------|--------------|---------------|--------------|-----------------------------|----------------|-------|----------------|-------|----------------|-------|----------------|
|               |              |               |              | 3,000                       |                | 4,000 |                | 5,000 |                | 6,000 |                |
|               |              |               |              | Min.                        | Percent<br>El. | Min.  | Percent<br>El. | Min.  | Percent<br>El. | Min.  | Percent<br>El. |
| 3.23          | 25.89        | Bal.          | 0.040        | 71.3                        | 7.0            | 19.9  | 6.8            | 13.6  | 6.5            | 2.5   | 7.5            |
| 4.77          | 26.34        | Bal.          | 0.003        | -----                       | -----          | 30.6  | 6.8            | ----- | -----          | 4.4   | 7.0            |
| 10.64         | 25.05        | Bal.          | 0.003        | -----                       | -----          | 26.4  | 6.5            | 15.5  | 6.5            | 5.25  | 5.5            |
| 15.61         | 23.76        | Bal.          | 0.040        | 153.9                       | 6.0            | 45.9  | 6.3            | ----- | -----          | 5.13  | 7.0            |
|               | 24.0         | Bal.          | 0.010        | -----                       | -----          | 45.7  | 10.0           | ----- | -----          | 10.2  | 9.3            |

TABLE V

| Percent<br>W | Percent<br>Ta | Percent<br>Cr | Percent<br>Mo | Percent<br>Al | Percent<br>C | Stress, p.s.i. at 1250° C. |                |       |                |       |                |       |                |
|--------------|---------------|---------------|---------------|---------------|--------------|----------------------------|----------------|-------|----------------|-------|----------------|-------|----------------|
|              |               |               |               |               |              | 3,000                      |                | 4,000 |                | 5,000 |                | 6,000 |                |
|              |               |               |               |               |              | Min.                       | Percent<br>El. | Min.  | Percent<br>El. | Min.  | Percent<br>El. | Min.  | Percent<br>El. |
| 23.76        | 10.64         | 10.68         | -----         | -----         | 0.040        | 153.9                      | 6.0            | 45.9  | 6.3            | 13.2  | 10.5           | 5.1   | 7.0            |
| 28.83        | 9.98          | -----         | -----         | -----         | 0.037        | 73.5                       | 11.5           | 26.9  | 10.0           | 13.9  | 12.0           | 7.1   | 10.0           |
| 26.26        | 10.28         | 11.61         | -----         | 1.57          | 0.071        | 71.38                      | 14.0           | 27.3  | 12.3           | ----- | -----          | 6.2   | 13.0           |
| 24.79        | 10.04         | 9.94          | -----         | -----         | 0.036        | 75.63                      | -----          | 33.8  | 13.0           | ----- | -----          | 10.2  | 11.5           |
| 24.29        | 8.84          | 9.47          | 10.04         | -----         | 0.036        | 37.5                       | 8.0            | 16.5  | 6.2            | ----- | -----          | 3.7   | 6.0            |

Table VI.—High heating tests on prior art alloys at temperature of 1250° C.

30

Table IX.—Results of standard creep-rupture tests on prior art alloys

| Weight percent composition                                             |       | Stress,<br>p.s.i. | Total<br>life, min. | Percent<br>elonga-<br>tion |
|------------------------------------------------------------------------|-------|-------------------|---------------------|----------------------------|
| 0.05 C, 22 Cr, 2.5 Co, Max., 6.5, 1.0 W,<br>2 Cr/Ta, 15 Fe, balance Ni | ----- | 3,000             | 1.3                 | 3.75                       |
| .2 C Max., 22 Cr, 2.0 Co, 9.0 Mo, 0.7 W,<br>18.5 Fe, balance Ni        | ----- | 3,000             | 6.7                 | 5.6                        |
| .25 C Max., 16 Cr, 6.5 Mo, 3.5 Ti, 10 Fe,<br>.25 Al, balance Ni        | ----- | 3,000             | 7.8                 | 9.5                        |
| .2 C Max., 21 Cr, 20 Ni 20 Co, 3 Mo, 2.5<br>W, 1 Cr/Ta, balance Fe     | ----- | 3,000             | 12.0                | 7.0                        |
| 0.5 C Max., 1 Cr, 2.5 Co, Max., 28 Mo, 5.5<br>Fe, balance Ni           | 40    | 3,000             | 18.9                | 4.3                        |

In addition, it has been found that a binary alloy of about 45 weight percent tungsten and the remainder nickel and incidental impurities exhibits surprising creep-rupture resistance as evidenced from the data in Table VII.

It should be noted that a comparison of the hour-life of the alloys of the present invention and prior art alloys under standard creep-rupture tests indicate that prior art alloys exhibit lives equal to or greater than the alloy of the present invention yet a comparison of minute-life of the present novel alloys (Tables II, III, IV and V) with

Table VII.—Influence of tungsten

| Percent<br>W | Percent<br>Ni | Stress, p.s.i. at 1,250° C. |                |       |                |       |                |       |                |       |                |
|--------------|---------------|-----------------------------|----------------|-------|----------------|-------|----------------|-------|----------------|-------|----------------|
|              |               | 2,000                       |                | 3,000 |                | 4,000 |                | 5,000 |                | 6,000 |                |
|              |               | Min.                        | Percent<br>El. | Min.  | Percent<br>El. | Min.  | Percent<br>El. | Min.  | Percent<br>El. | Min.  | Percent<br>El. |
| 44.91        | Bal.          | -----                       | -----          | 252.3 | 11.0           | 76.5  | 10.5           | 43.7  | 10.7           | 25.9  | 11.5           |
| 45.0         | Bal.          | -----                       | -----          | ----- | -----          | ----- | -----          | ----- | -----          | 10.5  | 9.3            |
|              |               |                             |                |       |                |       |                |       |                |       | 8.5            |

Table VIII includes data showing the results of conventional creep-rupture tests conducted on the alloys of the present invention. Table IX shows data resulting from conventional creep-rupture tests on prior art alloys.

60 the prior art alloys (Table VI) under rapid heating-creep-rupture tests indicates the surprising superiority of the present novel alloys.

When the alloy of this invention is to be employed in an oxidizing media, such as 10 percent boiling chromic acid, the addition of chromium to the base alloy in amounts up to 20 percent with the preferred range being about 10 percent, can reduce the corrosion rate to as little as 14.3 mils per year as shown in Table X and increase creep-rupture life as shown in Table V. In addition, where greater oxidation resistance is desired, for example, in cases where the alloy is subjected to high temperatures for periods of time measured in hours rather than in minutes, chromium may be added without substantially detracting from the superior properties of the base-alloy as noted in Table XI.

75 To further illustrate the versatility of the alloys of the

| Comp., percent       | Percent<br>C | Temp.,<br>°C. | Stress,<br>p.s.i. | Life,<br>hr. |
|----------------------|--------------|---------------|-------------------|--------------|
| 0 W, 10 Ta, Rem. Ni  | 0.002        | 982           | 5,000             | 2.8          |
| 5 W, 10 Ta, Rem. Ni  | 0.003        | 982           | 5,000             | 3.9          |
| 10 W, 10 Ta, Rem. Ni | 0.004        | 982           | 5,000             | 5.9          |
| 15 W, 10 Ta, Rem. Ni | 0.001        | 982           | 5,000             | 10.7         |
| 20 W, 10 Ta, Rem. Ni | 0.004        | 982           | 5,000             | 23.8         |
| 25 W, 10 Ta, Rem. Ni | 0.040        | 982           | 5,000             | 80.1         |
| 30 W, 10 Ta, Rem. Ni | 0.066        | 982           | 5,000             | 308.5        |
| 45 W, 10 Ta, Rem. Ni | 0.014        | 982           | 5,000             | 92.8         |

invention, corrosion resistance, oxidation resistance, and rapid heating tests were conducted on a chromium-containing and molybdenum-containing alloy of this invention.

An alloy consisting of 10.63 percent chromium, 9.99 percent tantalum, .25.83 percent tungsten, 0.037 percent carbon and the balance nickel and incidental impurities was subjected to corrosion tests in 10 percent boiling chromic acid. The average corrosion rate, given in mils per year, from five 48-hour periods was 14.3 as noted in the following Table X. The advantageous increase in corrosion resistance gained by the addition of molybdenum and iron are also shown in Table X.

Illustrated by reference to Table XII. Table XII shows the composition of three alloys cast under similar conditions into identical 3 inch molds. The significant differences between alloys 1, 2, and 3 is the carbon content.

5 Each ingot was lightly forged to insure that the cast structure had been sufficiently hot worked before heavier reductions were attempted.

Alloys 1 and 2 cracked severely during hot working. Alloy No. 2 cracked so quickly that almost no reduction in size was obtained. The alloy designated as 3 was hot worked to approximately a 1.000 inch slab. The forging

Table X

| Composition, weight percent |          |       |       |       |       |       | Corrosion rate, mils per year         |                         |                       |      |      |                 |                          |
|-----------------------------|----------|-------|-------|-------|-------|-------|---------------------------------------|-------------------------|-----------------------|------|------|-----------------|--------------------------|
| W                           | Ni       | Ta    | Cr    | Mo    | Fe    | C     | Boiling fuming nitric acid condensate | Boiling 65% nitric acid | Boiling sulfuric acid |      |      | Boiling 20% HCl | Boiling 10% chromic acid |
|                             |          |       |       |       |       |       |                                       |                         | 10%                   | 30%  | 55%  |                 |                          |
| 25.83                       | Bal..... | 9.99  | 10.63 | ----- | ----- | 0.037 | 5.0                                   | 9.1                     | 19.3                  | 47.0 | 113  | 863             | 14.3                     |
| 24.79                       | Bal..... | 10.04 | ----- | 9.94  | ----- | 0.036 | 3.30                                  | 9.30                    | 5.2                   | 27.1 | 116  | 229             | 142.0                    |
| 24.29                       | Bal..... | 8.84  | 9.47  | 10.04 | ----- | 0.036 | 7.70                                  | 31.70                   | 11.0                  | 60.0 | 217  | 630             | 22.9                     |
| 28.36                       | Bal..... | 5.36  | ----- | ----- | 5.08  | 0.005 | 2.98                                  | 15.7                    | 11.4                  | 56.9 | 14.3 | -----           | -----                    |
| 30.42                       | Bal..... | 9.94  | ----- | ----- | 9.22  | 0.010 | 0.91                                  | 2.37                    | 7.25                  | 30.4 | 67.4 | -----           | -----                    |

An oxidation resistance test was conducted on an alloy of the same composition as that subjected to the corrosion resistance test above. The oxidation test was conducted at 1900° F. for a period of 113 hours. At the end of this period, the oxidation rate, expressed as gain in weight in grams per square inch, was 0.01 as noted in Table XI.

Table XI

| Alloys of present invention, percent |       |       |       |       |          | Oxidation rate expressed as gain in weight in grams/sq. in./113 hrs. at 1900° F. |
|--------------------------------------|-------|-------|-------|-------|----------|----------------------------------------------------------------------------------|
| C                                    | W     | Ta    | Cr    | Al    | Ni       |                                                                                  |
| 0.027                                | 30.04 | ----- | ----- | ----- | Bal..... | 0.123                                                                            |
| 0.040                                | 25.89 | ----- | ----- | ----- | Bal..... | 0.115                                                                            |
| 0.012                                | 46.07 | ----- | ----- | ----- | Bal..... | 0.498                                                                            |
| 0.040                                | 23.76 | 10.64 | ----- | ----- | Bal..... | 0.142                                                                            |
| 0.037                                | 25.83 | 9.99  | 10.63 | ----- | Bal..... | 0.010                                                                            |
| 0.071                                | 26.26 | 10.28 | 11.61 | 1.57  | Bal..... | 0.014                                                                            |
| 0.080                                | 24.01 | ----- | 19.92 | 1.72  | Bal..... | 0.015                                                                            |

From these tests it can be seen that by the addition of certain other alloying materials to the nickel-base alloy certain desirable properties can be imparted to the alloy for certain specific purposes without substantially detracting from the very desirable combination of corrosion resistance, oxidation resistance, and high heating stress-rupture properties.

Iron may be present in the alloy of this invention in proportions as high as 10 percent by deliberate additions such as ferro-alloys, e.g., ferrotantalum. The results of such an addition are noted in Table X. However, for the best hot-working properties, the iron content, preferably, should not exceed the quantity introduced as an impurity in the usual melting operation, which is generally on the order of 1.5 percent. Although iron seems to increase corrosion resistance in some instances, it has the concurrent effect of decreasing amenability of the alloys to hot working.

Carbon, which is a conventional impurity, may be present in amounts up to a maximum of 0.5 weight percent. It is preferred however, that the carbon content be kept as low as possible. The carbon content of the alloy is particularly important with respect to the workability of the alloy. For the enhanced workability characteristics carbon contents of less than 0.15 are recommended. The most preferred alloys from the standpoint of workability are those which contain less than 0.12 weight percent carbon.

The influence of carbon content in workability is il-

lustrated by reference to Table XII. The significant differences between alloys 1, 2, and 3 is the carbon content.

Table XII

| Element         | 1     | 2     | 3     |
|-----------------|-------|-------|-------|
|                 |       |       |       |
| Tungsten.....   | 24.30 | 24.56 | 24.04 |
| Tantalum.....   | 8.07  | 8.96  | 9.38  |
| Chromium.....   | 9.28  | 9.55  | 9.38  |
| Molybdenum..... | 9.03  | 8.90  | 8.90  |
| Carbon.....     | 0.12  | 0.49  | 0.04  |

The alloy of this invention can be prepared by any of the well-known conventional methods. For example, the alloy may be prepared by induction melting the desired constituents in a vacuum furnace or under an atmosphere of an inert gas.

It may be seen that the unique combination of properties possessed by the alloy of this invention is very valuable in the missile field wherein at the present time from the best information available a service life of 15 seconds is adequate, whereas, under other conditions, a service life of 10 to 15 minutes may be required. The alloys of the present invention possess a creep-rupture life well in excess of the required life time presently thought to be required for missile service.

This application is a continuation-in-part of U.S. Serial No. 61,084, filed October 7, 1960 and now abandoned.

What is claimed is:

- An alloy consisting essentially of, along with incidental impurities, at least 25 weight percent nickel, 1 to 25 weight percent tantalum, 20 to 50 weight percent tungsten, a maximum of 0.15 weight percent carbon, and selected amounts of at least one metal chosen from the group consisting of iron, aluminum, molybdenum and chromium.
- An alloy consisting essentially of, along with incidental impurities, at least 40 weight percent nickel, 24 to 50 weight percent tungsten, 5 to 15 weight percent tantalum, a maximum of 0.15 weight percent carbon, and selected amounts of at least one metal chosen from the group consisting of iron, aluminum, molybdenum, and chromium.
- An alloy consisting essentially of, along with incidental impurities, at least 35 weight percent nickel, 20 to 45 weight percent tungsten, 1 to 20 weight percent tantalum, a maximum of 0.15 weight percent carbon, and selected amounts of at least one metal chosen from the group consisting of iron, aluminum, molybdenum, and chromium.
- An alloy consisting of about 25 weight percent tung-

sten, about 10 weight percent tantalum, about 10 weight percent chromium, less than about 0.50 weight percent carbon, the remainder nickel and incidental impurities.

5. An alloy consisting of about 25 weight percent tungsten, about 10 weight percent tantalum, about 10 weight percent molybdenum, less than about 0.50 weight percent carbon, the remainder nickel and incidental impurities.

6. An alloy consisting of about 25 weight percent tungsten, about 10 weight percent tantalum, about 10 weight percent chromium, about 10 weight percent molybdenum, less than about 0.50 weight percent carbon, the remainder nickel and incidental impurities.

7. An alloy consisting of about 30 weight percent tungsten, about 5 weight percent tantalum, about 5 weight percent iron, less than about 0.50 weight percent carbon, the remainder nickel and incidental impurities.

8. An alloy consisting of about 30 weight percent tungsten, about 10 weight percent tantalum, about 10 weight percent iron, less than about 0.50 weight percent carbon, the remainder nickel and incidental impurities.

9. An alloy consisting of about 25 weight percent tungsten, about 10 weight percent tantalum, about 10 weight percent chromium, about 2 weight percent aluminum, less than about 0.50 weight percent carbon, the remainder nickel and incidental impurities.

10. An alloy consisting of about 25 weight percent tungsten, about 10 weight percent tantalum, about 10 weight percent chromium, less than about 0.15 weight percent carbon, the remainder nickel and incidental impurities.

11. An alloy consisting of about 25 weight percent tungsten, about 10 weight percent tantalum, about 10

weight percent molybdenum, less than about 0.15 weight percent carbon, the remainder nickel and incidental impurities.

12. An alloy consisting of about 25 weight percent tungsten, about 10 weight percent tantalum, about 10 weight percent chromium, about 10 weight percent molybdenum, less than about 0.15 weight percent carbon, the remainder nickel and incidental impurities.

13. An alloy consisting of about 30 weight percent tungsten, about 5 weight percent tantalum, about 5 weight percent iron, less than about 0.15 weight percent carbon, the remainder nickel and incidental impurities.

14. An alloy consisting of about 30 weight percent tungsten, about 10 weight percent tantalum, about 10 weight percent iron, less than about 0.15 weight percent carbon, the remainder nickel and incidental impurities.

15. An alloy consisting of about 25 weight percent tungsten, about 10 weight percent tantalum, about 10 weight percent chromium, about 2 weight percent aluminum, less than about 0.15 weight percent carbon, the remainder nickel and incidental impurities.

#### References Cited by the Examiner

##### UNITED STATES PATENTS

|    |           |       |               |       |        |
|----|-----------|-------|---------------|-------|--------|
| 25 | 1,588,518 | 6/26  | Brace         | ----- | 75-174 |
|    | 1,807,554 | 5/31  | Rohn          | ----- | 75-171 |
|    | 1,836,317 | 12/31 | Franks        | ----- | 75-171 |
|    | 2,122,403 | 7/38  | Balke et al.  | ----- | 75-176 |
| 30 | 2,977,225 | 3/61  | Wlodek et al. | ----- | 75-176 |

DAVID L. RECK, Primary Examiner.

WINSTON A. DOUGLAS, Examiner.